

Patented June 24, 1924.

1,498,865

## UNITED STATES PATENT OFFICE.

CAMPBELL C. CARPENTER, OF NIAGARA FALLS, NEW YORK, ASSIGNOR TO U. S. LIGHT & HEAT CORPORATION, OF NIAGARA FALLS, NEW YORK, A CORPORATION OF NEW YORK.

### TREATMENT OF WOOD SEPARATORS.

No Drawing.

Application filed June 21, 1923. Serial No. 646,988.

To all whom it may concern:

Be it known that I, CAMPBELL C. CARPENTER, a citizen of the United States, residing at Niagara Falls, in the county of Niagara and State of New York, have invented new and useful Improvements in the Treatment of Wood Separators, of which the following is a specification.

This invention relates to the treatment of wood separators for storage batteries.

An object of the invention is to so treat a wood separator as to get the fibres of the wood in proper colloidal condition so as to more readily absorb and transfer sulphuric acid and so as to more readily diffuse battery acid.

A further object is to so prepare the separator that it will not be readily attacked by battery electrolyte, thereby increasing the separator life.

When the wood of the separator is in proper colloidal condition, it has the property of absorbing acid of greater density than that of the electrolyte surrounding it. This increases the conductivity of the separator.

In the process as outlined below, exact proportions and periods of time have been given as representing the best practice so far determined, but it is not intended that the stated proportions and time periods shall be construed as otherwise than illustrating

the principles of the process, it being understood that variations in proportions and details of treatment may be resorted to without departing from the principles of the invention as defined in the appended claims.

In the process herein described, Port Orford cedar has been employed, since it has been found that this wood is specially adapted for the manufacture of separators.

In carrying out the process, the separators cut to size, are placed in a supersaturated solution of lime and subjected to a pressure of thirty pounds per square inch or over in the presence of  $\text{SO}_2$  gas and heated for a period of approximately five hours.

What I claim as new and desire to secure by Letters Patent of the United States is:—

1. The process of preparing wood for use in battery separators which comprises treatment in a solution of lime by  $\text{SO}_2$  gas under heat and pressure.

2. The process of preparing wood for use in battery separators which comprises treating the wood in a supersaturated solution of lime with  $\text{SO}_2$  gas under pressure of approximately thirty pounds per square inch or over and heating for approximately five hours.

In witness whereof, I have hereunto subscribed my name.

C. C. CARPENTER.